

F. K. FISH, JR.

## PROCESS OF DRYING LUMBER

APPLICATION FILED JAN. 18, 1918. RENEWED AUG. 13, 1919.

1,328,507.

Patented Jan. 20, 1920.

3 SHEETS—SHEET 1.



Frederick K. Fish, Jr.,

By C. H. Ferguson

Attorney

F. K. FISH, JR.

PROCESS OF DRYING LUMBER.

APPLICATION FILED JAN. 18, 1918. RENEWED AUG. 13, 1919.

1,328,507.

Patented Jan. 20, 1920.

3 SHEETS—SHEET 2.



Fig. 4.



Fig. 5.

Inventor  
Frederick K. Fish, Jr.

By W. H. F.

Attorney

F. K. FISH, JR.

PROCESS OF DRYING LUMBER.

APPLICATION FILED JAN. 18, 1918. RENEWED AUG. 13, 1919.

1,328,507.

Patented Jan. 20, 1920.

3 SHEETS—SHEET 3.



Attorney

# UNITED STATES PATENT OFFICE.

FREDERICK K. FISH, JR., OF NEW YORK, N. Y.

## PROCESS OF DRYING LUMBER.

1,328,507.

Specification of Letters Patent. Patented Jan. 20, 1920.

Application filed January 18, 1918, Serial No. 212,467. Renewed August 13, 1919. Serial No. 317,392.

To all whom it may concern:

Be it known that I, FREDERICK K. FISH, Jr., a citizen of the United States of America, residing at 2 Stone street, New York city, in the county of New York and State of New York, have invented certain new and useful Improvements in Processes of Drying Lumber, of which the following is a specification.

10 This invention relates to improvements in a process for drying and treating wood. In my companion application for Patent Serial Number 261,938, renewed November 9th, 1918, I have described and claimed a 15 process for treating wood, in which the wood is subjected to a partial vacuum to expel a part of the air previous to the step of treating the wood in superheated water; the water in the early case being boiled previous to its introduction to the container; and the wood was finally treated in an equalizing chamber, and there dried.

It has been found to be advantageous to 25 preliminarily treat the green wood to a sweating step, previous to subjecting it to the action of the water, and it has also been demonstrated that if the water is superheated previous to its introduction to the container, quicker and more effective results are 30 obtained. Furthermore, to expedite the final drying, and to insure against checking the wood under differing climatic and atmospheric conditions, I have provided a cooling step.

35 Therefore one of the principal objects of the present invention is to provide a preliminary step to heat and soften the green wood, and otherwise put it in good condition to render it more susceptible to the water treatment. In this preliminary step, the green wood is placed in a substantially closed sweating chamber in which steam has been introduced to create a moderately heated moist atmosphere to raise the temperature of the wood throughout without danger of checking, and to soften the structure, open up the pores, dissolve the gummy sap matters and tend to free them from their confinement. This step in the process is continued long enough to cause the heated moist atmosphere to thoroughly permeate the entire wood structure and the warmth and moisture render the wood soft and pliable.

50 This treatment creates in the interior of the wood a high temperature, and while in this condition, the wood is removed to a

closed container, and is subjected to a vacuum, which expels a portion of the moisture, and otherwise conditions the structure for the action of the water.

60 Next the wood is subjected to the action of superheated water, to expel the gummy sap matters, and melt the contained resins. It has been found advantageous, both as to effect and expediency to superheat the water previous to introducing it to the wood. The interior of the wood at the time the water is introduced is highly heated and its structure is materially softened, consequently when the superheated water is introduced into the container, it promptly penetrates the wood structure without liability of internal checking, and the gummy sap matters are attacked and immediate dissolution commences. This is due to the fact 75 that the water is under pressure, and is heated above the boiling point, and as the wood structure is heated and otherwise in permeable condition, the water soluble gums and the resins are attacked without loss of time. 80

The previously heated wood and superheated water, therefore accomplishes two things, i. e., saves loss of time in treating the wood; and avoids all possibility of internal checking, accomplishments which have 85 decided advantages in producing practical results.

90 The cooling or tempering step in the present invention is one which adds materially to the effective curing or seasoning of the wood. For instance after the wood is removed from the equalizing chamber, the major portion of its water soluble matter is removed, and its contained resins are distributed throughout the wood structure, and 95 its interior is highly heated. The new substantially reconstructed wood structure is liable to surface cracking when removed to the air, due to the differences between the internal and external temperature, and to 100 avoid this possibility, the wood, according to the present invention is gradually cooled or tempered, to avoid the setting up of unequal stresses. This step is continued until about the time the internal and external temperature becomes equalized, which results in the resins setting in the spaces in the wood, previously occupied by the water soluble substances, without the wood in anywise checking or cracking.

105 110 In the foregoing description I have only emphasized the new steps in the present im-

provement, the entire process being herein-after described in detail.

Structurally, wood consists mainly of cellulose with its incrusting layers of lignin, and sap containing water, resins, tannins, coloring matter with other organic substances, together with a minor proportion of mineral matter or ash. Lignin, while not fully understood chemically, is closely allied to the cellulose of the wood, and since it forms a part of the permanent structure of the wood, it may, for purposes of the present invention, be regarded as identical with the cellulose.

15 Of the other organic substances, the principal are starches, gummy substances and albuminous compounds found in the watery sap and in the wood structure, together with resins or resinous compounds mainly to be found in the resin cells or ducts. The starches, gums and albuminous substances with the watery sap are elements principally necessary to the life of the growing tree but their presence in felled wood, timber or lumber, if in any quantity, is largely detrimental as affording principal elements leading to the decay or destruction of the wood. Therefore, any proper treatment of the wood to preserve the same should be directed to the removal of the starches, gums, albuminous substances and sap water with the proper preservation of the resins and resinous substances and the distribution of the same throughout the structural elements, care being taken to the end that the wood is not kept under treatment long enough to disintegrate or destroy the wood as such, so that the elasticity, strength and that which is termed "life" is removed.

In carrying out my improved process, certain steps are provided to utilize the natural bases of the resins, acetic acid and tannic acid existing in the wood, as preservative agents; that is to say, these constituents or substances are dislodged from their cellular confinement, and separated from their original vehicle, the water soluble constituents being dissolved, and the major portion removed from the wood, the remainder being distributed through, and deposited upon the fibrous structure of the wood.

With a full appreciation of the structure of wood, the various steps in the process are designed to expel the water soluble constituents, and replace same with the contained resins, to insure of the proper treatment and drying of the wood, without cracking, checking or other physical deterioration. Wood treated according to the improved process is substantially non-hydroscopic, and correspondingly immune from spores, or fermentation or the like, and undergoes the minimum amount of shrinkage.

To illustrate one way of carrying out the process, reference is made to the accompanying drawings, wherein:

Figure 1 is a vertical longitudinal section of a sterilizer, suitable for carrying out certain of the steps of the process.

Fig. 2 is a diagrammatic illustration of the apparatus associated with the sterilizer for controlling it.

Fig. 3 is a transverse section of the sterilizer.

Fig. 4 is a vertical longitudinal section of an equalizing chamber.

Fig. 5 is a section on the line 5—5, Fig. 4.

Fig. 6 is a diagrammatic plan view of the various containers, showing their means of intercommunication.

Fig. 7 is a side elevation of the same.

1 represents a sterilizer of construction suitable for containing superheated water, and is preferably provided with a presser plate 2, with means for adjusting same, such for instance as screws 3. By this means the charge of wood may be kept under pressure and prevented from floating, or becoming distorted while being treated. The container or sterilizer is provided with heating coils 4, by which the temperature of the atmosphere, steam or water within may be heated to the desired degree; and perforated coils 5 are provided for the purpose of supplying steam within the container when desired.

To equip the sterilizer 1 for conveniently developing the several conditions incident to the different steps of the process, it is provided with an exhaust pipe 6 leading to a vacuum pump, 7 with an interposed condenser 8; a water supply pipe 9 that communicates with a vertical pipe 10 leading to an elevated water supply tank, and also with a pump 11, by means of which water once supplied to the sterilizer 1, may be withdrawn, and for the sake of economy, returned to the elevated tank for reuse. Water supplied through pipes 9 and 10 to the sterilizer 1, will preferably be previously superheated and the coils 4 relied upon for maintaining its heat or raising it to the proper degree. The pipes 6, 9 and 10, as well as the connections with the return pipe for the water, are provided with suitable valves to open and close them appropriately to the several steps of the process. 12 represents tracks to receive the car or truck upon which the wood is loaded for introduction into the sterilizer.

Referring to Figs. 4 and 5, 13 represents the equalizing chamber which is preferably provided with a pressure device 2<sup>a</sup>, 3<sup>a</sup>, similar in principle to that employed in the sterilizer 1, with heating pipes 14 preferably located at the bottom, an air inlet or damper 15, and an air outlet or damper 16. This

equalizing chamber is further provided with tracks 17 for convenient introduction of the charge of wood, and its walls are preferably constructed so as to have a high co-efficient of heat insulation for the sake of economy in operation.

Referring to Fig. 6, 18 represents the sweat chamber; 19 a transfer platform for transferring a truck load of wood to equalizing chambers 20, when withdrawn from sterilizer 1; 21 are tracks upon which platform 19 is adapted to travel; and 22 are cooling or tempering chambers. Equalizing chambers and cooling chambers 20 and 22 respectively, are provided with tracks 23, extending therethrough for the convenient introduction thereinto of a truck load of wood. 17 is a track extending through sweat chamber 18, sterilizer 1, and transfer platform 19, for the convenient introduction therethrough of a truck load of wood.

In carrying out the process with the apparatus above described, a charge of wood is loaded on a truck, and is introduced into the sweat chamber 18, the sweat chamber having previously had created therein a moderately heated moist atmosphere, steam being employed for this purpose. The wood having been introduced to the moist atmosphere, the chamber is closed and the wood is subjected to the moist heat until it becomes heated and saturated throughout its entire structure. The moist atmosphere penetrates the fibrous structure and softens the wood, sweats the fibers, and opens up the pores, and tends to soften the sap matter and resins.

The wood is retained in the sweat chamber sufficient time to insure of it being internally heated throughout, and well conditioned for future treatment. The wood is removed from the chamber, and while in a heated condition, and well moistened, it is quickly introduced into the container or sterilizer 1, the pressing devices are operated to hold down the wood and then the container is hermetically sealed. A partial vacuum is now created in the container, the vacuum pump 7 being operated to accomplish this function.

The partial vacuum is continued for sufficient time to evaporate a portion of the aqueous content of the wood, without taking with it the resins or the resin-producing constituents. Superheated water is now introduced into the container to completely submerge the wood, the water being forced in either by pressure from the tank above, or by operating the pump 11. The wood remains in the water for approximately one hour, and pressure of about twenty pounds is maintained. The pressure is provided by the pump 11, and is maintained by continuing the heating through means of the heating coils 4.

In this step of the process, the super-

heated water commences to act immediately on the wood, as the latter, it will be remembered has been previously heated and softened, and is favorable for prompt action of the water. The highly heated water under 70 pressure, is forced through the wood structure, and the gummy sap matter is dissolved and mixed with the water, and consequently is displaced and removed from the wood. The resins are also subjected to the heated 75 water, and readily melt and spread throughout the wood, taking the place of the displaced and dissolved gummy sap matter. The individual fibers are swelled or enlarged by the action of the water, heat and pressure 80 without in anywise checking or cracking the structure, and in addition the confined water causes a deposition of the colloidal substances of the fibers of the wood, and tans the surface of the latter, giving the wood a distinctive appearance.

After the wood is subjected to the superheated water, the valves are manipulated, and the pressure in the container, or the pump 11 may be employed, forces the water 90 back into the tank and it may be reused. A second vacuum is now created, preferably of about twenty inches, and for a period sufficient to expel or evaporate a greater portion of the moisture content of the wood, 95 and without taking with it the values of the sap, such as the resins and resin producing substances.

To continue the withdrawal of the moisture from the interior of the wood and prevent cracking and checking, the second mentioned vacuum is gradually replaced by an artificial atmosphere of high temperature, say about 290° F. This condition is created 100 by introducing steam to the container 105 through the perforated pipes, the temperature being kept up by passing steam through the heating coils 4. Some pressure is maintained during this time—say about thirty pounds—and the step is continued for—say 110 half an hour. The action of the same, heat and pressure, has the effect of restoring the internal temperature of the wood well above the boiling point and keeping the retained values of the sap, and resins in good permeating condition.

Next the steam is cut off from the perforated pipes, and while the wood is favorable to giving up moisture, is again subjected to a partial vacuum of about fifteen 120 inches. This step is continued for about two hours, but the vacuum may be increased toward the end of the step, say for the last half-hour thereof. This vacuum has the effect of aiding in uniformly distributing the 125 resins through the wood structure, and when completed, the wood is in condition to be removed from the sterilizer.

The load of wood is now rapidly transferred to the equalizing chamber. When in 130

this chamber the wood is subjected to an atmosphere at a temperature sufficient to cause continuous evaporation of moisture through the entire structure, at the same time keeping 5 the retained resins and resin substances in a melted condition. This is accomplished by passing steam through the coils 14, and at the same time a current of heated air is periodically forced through the chamber by 10 means of pipes (not shown), or by operating the dampers 15 and 16.

Upon the first introduction of the wood in the chambers, the dampers 15 and 16 are closed and the evaporated moisture rapidly 15 creates a humid condition within the chamber. As the humidity increases moisture occurs on the surface of the wood, and as the point of saturation is approached, evaporation 20 of the moisture ceases. At such time the dampers are operated to relieve the condition within the chamber, and this may be secured either by opening the upper damper alone, or by periodically opening both dampers, or introducing a separate current of 25 air around the wood, which accelerates the evaporation of the moisture, as fully set out in my co-pending application for patent above identified.

During the treatment of the wood in the 30 equalizing chamber, the melted resins permeate the cellulose, and are caused to spread into the places previously occupied by the water soluble constituents, and it is now that the next and final step is brought in to insure 35 against checking or cracking when bringing the wood to atmospheric temperature.

After treatment in the equalizing chamber, the wood is quickly conveyed to the 40 cooling or tempering chamber. This chamber is preferably of sufficient size to take a number of loads of wood, and as a load or loads is or are removed to the atmosphere, the others are advanced toward the exit.

45 Steam is introduced to the cooling chamber to create a moist moderately heated atmosphere which is so regulated as to allow of the gradual reduction of the internal temperature of the wood; as moisture evaporating 50 from the wood, together with the steam creates a humid condition around the wood, which is harmonized with the internal temperature, which results in a gradual setting of the distributed resins. This step is kept 55 up sufficient time to bring the temperature of the wood to atmospheric temperature, consequently the wood is artificially dried throughout, and when moved out into the atmosphere it will not check or shrink and 60 the resins will be set.

From the foregoing description it will be seen that the improved steps in the process will greatly facilitate the treating and drying of the wood. The step of sweating the 65 wood saves considerable time in completing

the process as it is evident the fibrous structure will be more susceptible to the action of the superheated water, and the latter will at once dissolve and remove the water soluble constituents, and melt the resins. Furthermore the cooling or tempering step will so gradually reduce and harmonize the temperature of the wood with that of the atmosphere that the resins in setting during the final drying will not shrink, crack or 75 check the wood structure.

What I claim is:—

1. The process of treating wood which comprises applying to wood water in a superheated condition, then submerging the 80 wood therewith, and permeating the wood throughout and arresting the treatment and removing the water before any substantial destruction of the fibers occurs to remove the major portion of the fermentable substances. 85

2. The process of treating wood which comprises superheating liquid and applying the liquid while superheated to wood which has been preheated to sweat the same, and submerging the wood therewith, to permeate the 90 wood throughout.

3. The process which comprises superheating liquid which has been previously used in the wood treatment, applying the liquid while superheated to wood, preheated to a 95 temperature to receive the superheated liquid without danger of checking or cracking, submerging the wood therewith, and removing the superheated liquid.

4. The process which comprises superheating liquid which has been previously used in wood treatment, applying the liquid while superheated to wood, submerging the wood therewith, and removing the superheated liquid. 100

5. The process of treating and drying wood which comprises softening its structure, then dissolving and removing from the softened wood water soluble constituents, and then drying the wood at a temperature 110 sufficient to induce ready evaporation and to permit the spreading of the resins to permeate the fibers of the wood. 105

6. The process of treating wood comprising sweating the wood to soften it, submerging 115 the wood in liquid to dissolve and extract the soluble gums and sap, and then subjecting the wood to a temperature to induce evaporation of the moisture of the wood and prevent hardening of the resins to permit 120 the spreading of the resins to permeate the fibers of the wood.

7. The process of treating wood comprising sweating the wood to soften it and raise the temperature therein, subjecting the wood 125 to the action of a vacuum, thereafter submerging the wood in liquid under pressure, and then again subjecting the wood to the action of a vacuum.

8. The process of treating wood compris- 130

5 ing sweating the wood to soften it and raise the temperature therein, subjecting the wood to the action of a vacuum, thereafter submerging the wood in liquid under pressure, then again subjecting the wood to the action of a vacuum, and finally drying the wood.

9. The process of treating wood which comprises preheating wood to sweat it and applying to and surrounding the wood while in such heated condition with superheated water, which has similarly been used, removing the superheated water and consequently drying the wood.

15 10. The process of drying wood comprising preheating the wood to sweat it, then subjecting the wood to superheated water and subsequently subjecting the wood to heat at a temperature sufficient to induce evaporation and prevent hardening of the resins.

25 11. The process of treating wood which comprises preheating wood to sweat it and applying to and surrounding the wood while in such heated condition with superheated water, removing the water, and subsequently drying the wood.

30 12. The process of treating wood which comprises preheating wood applying to and surrounding the wood with superheated water, which has been similarly used, removing the superheated water and subsequently subjecting the wood to a temperature sufficient to induce evaporation of the moisture 35 in the wood and prevent hardening of the resins thereby causing the resins to permeate the fibers of the wood.

40 13. The process of treating wood comprising subjecting the wood to the action of a vacuum to remove the air therefrom, then submerging the wood in fluid under pressure to dissolve and extract the soluble gums and sap, subsequently drying the wood, and thereafter conditioning the wood.

45 14. The process of treating wood comprising subjecting the wood to steam to soften its structure, to prepare it for subsequent treatment, submerging the wood in liquid under pressure to remove the soluble 50 gums and sap, and subsequently subjecting the wood to a temperature to induce evaporation of the moisture of the wood and prevent hardening of the resins thereby causing the resins to permeate the individual 55 fibers of the wood.

15. The process of treating wood comprising subjecting wood to steam to soften its structure to prepare it for subsequent treatment, then submerging the wood in liquid under pressure to dissolve and extract the soluble gums and sap, then subjecting the wood to a vacuum, and finally drying the wood at a temperature to induce evaporation of the moisture of the wood and prevent hardening of the resins thereby caus-

ing the resins to permeate the fibers of the wood.

16. The process of treating wood comprising sweating the wood, then subjecting the wood to a vacuum, then subjecting the wood to heated water under pressure to extract the soluble gums and sap, then subjecting the wood to a vacuum, subsequently treating the wood with steam while applying dry heat, again subjecting the wood to a vacuum while applying drying heat, then subjecting the wood to heat, and finally conditioning the wood.

17. The process of treating wood comprising sweating the wood to soften and heat the same, submerging the wood in heated water, and subsequently subjecting the wood to a drying temperature to produce a wood having the major portion of its gummy sap and other readily fermentable matters removed and its preservative substances diffused throughout the wood.

18. The process of treating wood comprising sweating the wood to soften and heat the same, treating the wood to dissolve and remove water soluble constituents, and subsequently drying the wood.

19. The process of treating wood comprising sweating the wood to soften and heat the same, and submerging the wood in heated water under pressure to dissolve and remove water soluble constituents.

20. The process of treating wood comprising sweating the wood, then treating the wood to a vacuum, subjecting the wood to heated water, thereafter subjecting the wood to a drying temperature, and finally conditioning the wood.

21. The process of treating wood comprising subjecting the wood to a vacuum, subjecting the wood to heated water to dissolve and remove water soluble constituents, subsequently treating the wood to a drying temperature, and thereafter conditioning the wood.

22. The process of treating wood comprising supplying heat to the wood at a temperature sufficient to evaporate moisture therefrom and removing accumulating moisture from around the wood and thereafter removing the wood and subjecting it to a confined moist atmosphere while the temperature is being reduced to condition the same.

23. The process of treating wood comprising sweating the wood to soften and heat the same, then to a vacuum, then subjecting the wood to heated water to dissolve and remove the water soluble constituents, subjecting the wood to a vacuum, then to steam, then to a vacuum, subjecting the wood to a heated and moist atmosphere to evaporate moisture, and finally subjecting the wood to a confined moist atmosphere while the temperature is being reduced to condition the same.

24. The process of treating wood comprising subjecting the wood to a vacuum, then to heated water to dissolve and remove the water soluble constituents, subjecting the wood to a vacuum, then to steam, then to a vacuum, subjecting the wood to a heated and moist atmosphere to evaporate moisture, and finally subjecting the wood to a confined moist atmosphere while the temperature is being reduced to condition the same.
25. The process of treating wood comprising subjecting the wood to heated water to dissolve and remove the water soluble constituents, subjecting the wood to a vacuum, then to steam, then to a vacuum, subjecting the wood to a heated and moist atmosphere to evaporate moisture while removing excess moisture, and finally subjecting the wood to a confined moist atmosphere while the temperature is being reduced to condition the same.
26. The process of treating wood comprising subjecting the wood to a vacuum, then to steam, then to a vacuum, subjecting the wood to a heated and moist atmosphere to evaporate moisture, and finally subjecting the wood to a confined moist atmosphere while the temperature is being reduced, to condition the same.
27. The process of treating wood comprising sweating the wood to soften and heat the same, then subjecting the wood to a vacuum, then to heated water, then to a vacuum, and thereafter subjecting the wood to steam to evaporate moisture.
28. The process of treating wood comprising sweating the wood to soften and heat the same, then subjecting the wood to a vacuum, then to heated water, then to a vacuum, thereafter subjecting the wood to steam to evaporate moisture, and then to a vacuum.
29. The process of treating wood comprising sweating the wood to soften and heat the same, then subjecting the wood to a vacuum, then to heated water, then to a vacuum, thereafter subjecting the wood to steam to evaporate moisture, then to a vacuum, and thereafter subjecting the wood to a drying temperature while removing moisture from around the wood.
30. The process of treating wood comprising sweating the wood to soften and heat the same, then subjecting the wood to a vacuum, and thereafter submerging the wood in heated water to dissolve and remove water soluble constituents.
31. The process of treating wood while in a heated condition and of superficial dryness by subjecting it to a humid atmosphere approaching saturation and of substantially the temperature of the wood and gradually reducing the heat of the wood and the surrounding atmosphere while removing excess moisture, until the wood is uniformly conditioned.
32. The process of treating wood while in a heated condition and of superficial dryness by subjecting it to a humid and heated atmosphere of substantially the heat of the wood and gradually reducing the temperature, producing a drying of the interior of the wood and a proper conditioning of the same.
33. The process of treating wood comprising sweating the wood to soften and heat the same, then subjecting it to a vacuum, and thereafter subjecting the wood to a drying temperature in a moist atmosphere and periodically removing excess moisture.
34. The process of treating wood comprising sweating the wood to soften and heat the same, thereafter subjecting the wood to a drying temperature, and then subjecting the wood to a humid and heated atmosphere of substantially the heat of the wood and gradually reducing the temperature, producing a drying of the interior of the wood and a proper conditioning of the same.
35. The process of treating wood comprising sweating the wood to soften and heat the same, then subjecting the wood to a vacuum and heat to evaporate moisture, thereafter subjecting the wood to steam under pressure, and finally drying the wood.
36. The process of treating wood comprising sweating the wood to soften and heat the same, then subjecting it to a vacuum and heat to evaporate moisture and thereafter subjecting the wood to a humid and heated atmosphere of substantially the heat of the wood and gradually reducing the temperature producing a drying of the interior of the wood and a proper conditioning of the same.
37. The process of treating wood comprising sweating the wood to soften and heat the same, thereafter subjecting the wood to heat under pressure to evaporate moisture, thereafter drying the wood in a moist atmosphere and periodically removing accumulating moisture.
38. The process of treating wood comprising subjecting the wood to a vacuum and heat to expel air therefrom, thereafter subjecting the wood to a drying temperature, and finally subjecting the wood to a humid and heated atmosphere of substantially the heat of the wood and gradually reducing the temperature, producing a drying of the interior of the wood and a proper conditioning of the same.
39. The process of treating wood comprising sweating the wood to soften and heat the same, submerging the wood in heated water under pressure to dissolve and remove the water soluble constituents removing the water, and thereafter drying the wood at about atmospheric pressure and in the presence of heat while introducing a current of heated air.

70

75

80

85

90

95

100

105

110

115

120

125

130

40. The process of treating wood comprising subjecting the wood to a vacuum to expel a portion of the air therefrom, treating the wood to soften its structure and dis-  
5 solve gummy sap matter, then to a vacuum, and then subjecting the wood to heat at about atmospheric pressure while periodically removing the accumulating moisture surrounding the wood while introducing a  
10 current of heated air.
41. The process of treating wood comprising sweating the wood to soften and heat the same, then subjecting the wood to a vacuum, then submerging the wood in superheated water to dissolve and remove water soluble constituents, and thereafter drying and conditioning the wood.
42. The process of treating wood comprising sweating the wood to soften and heat the same, thereafter submerging the wood in superheated water to dissolve and remove water soluble constituents, removing the water from around the wood, and then subjecting the wood to a vacuum to withdraw moisture therefrom.
43. The process of treating wood comprising preheating the wood, submerging the wood in superheated water to dissolve and remove water soluble constituents, removing the water and subsequently subjecting the wood to a drying heat.
44. The process of treating wood comprising preheating the wood, submerging the wood in superheated water to dissolve and remove water soluble constituents, removing the water, and then subjecting the wood to a plurality of vacuum treatments alternated with a pressure around the wood, and thereafter subjecting the wood to a drying heat.
45. The process of treating wood comprising sweating the wood, thereafter submerging the wood in superheated water to dissolve and remove water soluble constituents,
- removing the water, then subjecting the wood to a plurality of vacuum treatments alternated with a raising of the pressure around the wood, the temperature of the wood during these steps being maintained up to a degree sufficient to induce evaporation and prevent hardening of the resins, finally conditioning the wood in a moderately heated moist atmosphere.
46. The process of treating wood comprising sweating the wood to soften and heat it, thereafter submerging the wood and treat-  
55 ing it in superheated water to dissolve and remove water soluble constituents, removing the water, and thereafter surrounding the wood by a body of moderately heated moist atmosphere.
47. The process of treating wood comprising sweating the wood to soften and heat it, subsequently creating around the wood a body of steam under pressure to permeate the same and evaporate a portion of the moisture, and subsequently subjecting the wood to drying heat while removing excess moisture from around the wood.
48. The process of treating wood comprising sweating the wood to soften it, there-  
70 after treating the wood to dissolve and remove water soluble constituents and evaporating moisture under vacuum and in a moist atmosphere and causing the retained resins to spread throughout the wood structure.
49. The process of treating wood comprising sweating the wood to soften it, then alternately subjecting the wood to vacuum and super-heated water to dissolve and remove water soluble constituents and evapo-  
80 rate moisture, and subsequently treating the wood in a heated moist atmosphere and removing excess moisture while drying.

In testimony whereof I affix my signature.

FREDERICK K. FISH, JR.